

S. U. S. Patent  
Office  
Specimen

## UNITED STATES PATENT OFFICE.

BARBRA DIRNBERGER, OF SYRACUSE, NEW YORK, ADMINISTRATRIX OF  
JOHN DIRNBERGER, DECEASED, ASSIGNOR TO MICHAEL HEMMER, OF  
SAME PLACE.

## WALL-PLASTER.

SPECIFICATION forming part of Letters Patent No. 494,981, dated April 4, 1893.

Application filed July 11, 1892. Serial No. 439,712. (No specimens.)

*To all whom it may concern:*

Be it known that I, BARBRA DIRNBERGER, a citizen of the United States, residing in the city of Syracuse, county of Onondaga, and 5 State of New York, administratrix of the estate of JOHN DIRNBERGER, a late citizen of Syracuse, New York, deceased, hereby assert that the said JOHN DIRNBERGER, deceased, did invent a new and useful Improvement in *Composition for Wall-Plaster*, of which the following is a specification.

The invention relates to quick setting wall plaster.

The object is to produce a quick setting wall 15 plaster, adapted to be used where it is desired to finish up quickly and without having to wait for the same to dry as is the case in common mortar wall plaster.

The invention consists in mixing and combining the several ingredients hereinafter set forth in substantially the proportion specified, although not confined to these exact proportions, as it will be evident that they may be varied without materially departing from 20 the spirit of the invention.

For a batch of plaster containing about five hundred and eighty (580) pounds use the following ingredients. First take four hundred pounds of hydrated sand, one hundred and 25 twenty pounds of plaster of paris, and forty pounds of slaked lime. This is called the base,

which is first very thoroughly mixed together. To this is added what may be called a chemical, twenty pounds, the ingredients of said chemical being fully set forth in the application filed simultaneously herewith, and consisting of 35 muriatic acid, Glens Falls lime, soluble glass and glue water. By Glens Falls lime is meant lime which is very pure, it containing about ninety-five per cent. lime, one per cent. magnesia and one per cent. silica. To this composition may be added acellulose of vegetable matter, for the purpose of imparting a certain elasticity to the wall plaster after it has been put on. When it is desired to use the plaster, it 40 is mixed with water to a plastic condition and put on in the usual way.

Having described this invention, what is claimed is—

The herein described wall plaster, consisting of sand, plaster of paris, slaked lime, muriatic acid, lime, soluble glass, glue water and tissues of fiber, as set forth.

In witness whereof I have hereunto set my hand this 25th day of June, 1892.

BARBRA DIRNBERGER,  
*Administratrix of the estate of John Dirnberger, deceased.*

Witnesses:

E. O. JOHNSON,  
HOWARD P. DENISON.